# EUROPEAN PATENT SPECIFICATION

(11) **EP 1 266 040 B1**
(45) Date of publication and mention of the grant of the patent: **22.09.2004**
(21) Application number: 99962502.3
(22) Date of filing: 01.11.1999
(51) Int. Cl.: C14C 11/00

(54) **A TRANSFER MEMBER FOR IMPARTING A FINISH LEATHER**
SPRITZGEGENSTAND ZUM VEREDELN VON NACHBEARBEITETEM LEDER
ELEMENT DE TRANSFERT PERMETTANT DE CONFERER UN ASPECT FINI A DU CUIR

(43) Date of publication of application: 18.12.2002
(73) Proprietor: Max India Limited, Punjab (IN)
(72) Inventor: KAUSHIK, Pushpinder, Kumar, Chandigarh 160 022 (IN)
(74) Representative: Petersen, Frank, Dipl.-Ing.
(86) International application number: PCT/IN1999/000058
(87) International publication number: WO 2001/032938

(56) References cited:
- DE-A- 3 401 677
- GB-A- 2 002 260
- PATENT ABSTRACTS OF JAPAN vol. 17, no. 497 (M-1476) 08 September 1993 & JP 05 124 394 A (TOPPAN PRINTING CO LTD) 21 March 1993

## Description

This invention relates to a transfer member for treatment of leather so as to impart gloss properties thereto.

### PRIOR ART

It is generally known that hide is subjected to a chemical treatment to produce leather. However, if an appearance or finish is required, it was hitherto necessary to subject leather to an additional step of chemical treatment so as to impart a gloss appearance. It would be apparent that such a known process had the disadvantage of an additional step of chemical treatment.

A further disadvantage of the known art is that associated with split leathers. In accordance with the known art, split leather was subjected to 'the step of lamination, pigmentation or transfer foil so as to upgrade or improve the quality of split leather. Thus, split leather is impregnated with binder and waxes so that when compressed a release takes place from the plate. After impregnation it is then laminated, pigmented or treated with a transfer foil. A disadvantage is that the fiber bundles do not get concealed and continue to be in a standing position.

A transfer foil is disclosed in JP-A- 05 124 394. This is constituted of a base film, peeling layer and colouring adhesive layer. This prior art relates to applying design to artifical leather or synthetic leather.

Yet another known disadvantage is that of the chemical adhering to the plate.

### OBJECTS OF THE INVENTION

An object of this invention is to propose a transfer member for treatment of leather and so as to impart gloss properties thereto.

Another object of this invention is to propose a transfer member for treatment of leather and so as to provide a uniform feel to leather.

Still another object of this invention is to propose a transfer member for treatment of leather and which provides good plate releasing properties.

Yet another object of this invention is to propose a transfer member for treatment of leather and which provides a good sealing of fibers.

A further object of this invention is to propose a transfer member for treatment of leather and which provides grain flatness.

Another object of this invention is to propose a transfer member for imparting a gloss together with a colour, print or metallic finish to leather.

### DESCRIPTION OF INVENTION

According to this invention there is provided a transfer member for imparting gloss properties to leather comprising a gloss film of at least two co-extruded layers and, wherein, the inner layer is the active or gloss layer and the outer layer is a colayer, a carrier or substrate layer releasably held to said outer layer.

The gloss film preferably comprises three coextruded layers and wherein the inner layer has the gloss properties, an intermediate layer is the colayer which contributes to the bulk properties of the film and further is a storage layer for the migratory chemicals, and an outer layer which is a colayer. A carrier such as paper is adhered to the outer layer.

Further preferred embodiments are defined in dependent claims 3-21.

The inner layer comprises a resin layer of isotactic polypropylene alone or in combination with random ethylene propylene copolymer present in an amount of 0 to 40% by weight. The intermediate layer comprises isotactic polypropylene and migratory additives, which are antistatic and slip agents. The outer layer also comprises isotactic polypropylene with an additive, which is an antiblock agent. A stiffener such as paper is adhered to the outer layer by means of an adhesive.

The inner layer may additionally comprise migratory chemicals present in the amount of 0-5%, migratory chemicals being antistatic and slip agents selected from erucamide stearamide, silicon oil, stearic acid and stearates used alone or in any combination thereof. Further, the inner layer may comprise an antiblock agent present in the amount of 500-4000 PPM. The antiblock agents are selected from silica, silicate, clay, talc and quartz alone or in any combination thereof. The haziness or glossyness of the inner layer is varied by changing the thickness of the inner layer and quantity of migratory chemicals and antiblock agents in the composition.

The migratory chemicals comprising said antistatic and slip agents are present in the amount of 500-10000 PPM by weight in the intermediate layer.

The outer layer is identical to the inner layer and comprises isotactic polypropylene in combination with random co-polymer of ethylene propylene, and where ethylene propylene is present in the amount of 0 to 40% by weight. The film further comprises a paper layer adhered to the outer layer. The paper layer is a cellulosic paper such as cromo art paper and having a grammage of 30 to 100 g/m².

The isotactic polypropylene present in the layers has an average molecular wt. of 25000 to 1,000,00, a melt flow index of 1-25 at 230°C/2.16 kg and density of 0.892 to 0.92.

As herein described -above an antiblock agent is provided in the outer layer. However, in the instance of a film having three layers, the antiblock agent may or may not be provided in the outer layer. In accordance with another embodiment, an antiblock agent is provided in the outer and in the inner layer. The outer layer may be subjected to a corona treatment, flame treatment or chemical treatment so as apply an adhesive thereon to secure a paper layer therewith. The paper layer acts as a stiffener and absorbs excess heat during the plating of the leather.

The transfer member of the present invention has a thickness of 8-45 x 10⁻⁶ m (8 to 45 microns). If the thickness is greater than 45 x 10⁻⁶ m (microns), it does not affect the workability or properties of the film, but no advantages are derived therefrom and only adds to the end cost of the film. If the thickness is less than 8 x 10⁻⁶ m (microns), the required quality and properties are then not achieved. Both the inner and outer layers should have sufficient thickness in the instance of two layers film, in order to store and release the chemicals therefrom. Similarly, the inner, intermediate and outer layers should have sufficient thickness in a three layers structure for storage and release of said chemicals. Preferably the transfer member has a thickness of 12-45x10⁻⁶ m (12 to 45 microns).

The inner and intermediate layers have each a thickness of 2-8x10⁻⁶ m (2 to 8 microns) and preferably a thickness of 2-5x10⁻⁶ m (2 to 5 microns). If the thickness of the inner layer is less than 2x10⁻⁶ m (microns), then gloss would reduce. If the thickness is more than 8x10⁻⁶ m (microns), and the outer, intermediate and inner layers are extruded then problems may arise in the coextrusion of the layers.

In the following table the properties of the gloss film are given in comparison with the predetermined specifications.

| COMPARISON PROPERTIES OF GLOSSY FILM | | | | | | |
|---|---|---|---|---|---|---|
| S.No. | PROPERTIES | UNIT | SPEC | ACTUAL RESULTS | SPEC | ACTUAL RESULTS |
| 1. | AVG.GAUGE | 10⁻⁶ m (MICRONS) | 15 | 14.9 | 2.0 | 20.1 |
| 2. | HAZE | % | 1.5 (MAX) | 1.2 | 1.5 (MAX) | 1.3 |
| 3. | GLOSS | | 95 (MIN) | 98 | 95 (MIN) | 97 |
| 4. | COEFFICIENT OF FRICTION | | | | | |
| | STATIC | | 0.55 | 0.50 | 0.45 | 0.56 |
| | DYNAMIC | | 0.55 | 0.48 | 0.55 | 0.54 |
| 5. | SHRINKAGE MD | % | 4.0 | 3.5 | 4.0 | 3.0 |
| | TM | % | 2.0 (MAX) | 1.0 | 2.0 (MAX) | 0.5 |
| 6. | TREATMENT | DYNES/CM | 38 (MIN) | 40 | 38 (MIN) | 40 |

Reference has been made hereinabove to a transfer member comprising only the gloss film on a carrier or substrate. The transfer member of the present invention also envisages, a transfer member having a foil in addition to the gloss film, said foil being selected from a colour, print or metallized foil.

In such an embodiment the transfer member comprises a carrier or substrate having the gloss film, the foil being provided on said film.

In each instance, the foil comprises of a plurality of layers with at least an outermost layer being an adhesive layer adapted to contact the leather surface, an inner most layer being a release layer in contact with the film and an active layer provided therebetween, and wherein the active layer is either a print, colour or metallized layer.

The colour foil further comprises a feel modifier layer with or without top protecting coat layer on said release coating, said colorant layer provided onto said feel modifier layer.

In the instance of a metallized transfer foil, the intermediate layers comprise a top coat layer on said release layer, said metallized layer being provided onto said top coat layer to provide metal finish to the leather.

The print foil intermediate layers comprise a feel modifier layer provide onto said release layer, a print coat layer provided onto said feel modifier layer. A top coat layer may or may not be provided on said feel modifier layer.

The feel modifier layer in itself comprises a plurality of layers. According to one embodiment, the feel modifier layer comprises at least two layers. One of said layers is a mixture of feel modifiers and a top coat or feel modifier and cover coat.

According to another embodiment the feel modifier layer comprises three layers namely a feel modifier layer adjacent to the release layer, a top coat layer adjacent to the feel modifier layer, and a covering layer adjacent the top coat layer.

The feel modifier layer comprises a combination of or only a single wax such as microcrystalline wax, paraffin, natural or synthetic waxes in solution or emulsion form. The waxes incorporated in the feel modifier imparts a waxy feel to leather.

According to an embodiment the feel modifier layer also comprises oils used alone or in combination with polydialkyl siloxane, olefin modified siloxanes, diethylene modified silicon oils, epoxy modified silicon oils, alcohol modified silicon oils.

According to another embodiment the feel modifier layer comprises a combination of waxes and lubricants as this also improves the scuff resistance properties. If a waxy feel is required, then the content of waxes present in the feel modifier layer is greater than that of the lubricants. However, if a silky feel is required then the content of lubricants present in the feel modifier layer is greater than the waxes. The feel modifier layer can consist of a combination of waxes and lubricants, or separate layers of waxes and lubricants.

The top coat layer is a protective coating for protecting the cover coat layer. The coat layer consists of lacquer and lacquer emulsions of various resins, such as nitrocellulose copolymer of vinyl chloride and vinyl acetate, polyurethane and polyamides with or without cross linking agents with or without fillers, such as silica.

The cover coat layer comprises essentially of natural resins such as shellac, caesin, albumin and gelatine or plasticizers. Alternatively, the cover coat layer may be selected from natural resins or synthetic resins such as acrylic, methacrylic, synthetic rubber, vinyl resin, nitrocellulose resins or polyurethane. In accordance with another embodiment, the natural resin may be present with the synthetic resin.

In accordance with yet another embodiment, the cover coat layer may also include colourants with or without dispersing agents, with or without cross linking or curing agents. The colourants may be selected from metallic pigments, pearl pigments of organic or inorganic nature or dyestuffs.

## Claims

1. A transfer member for imparting gloss properties to leather comprising a gloss film of at least two coextruded layers and, wherein, the inner layer is the active or gloss layer and the outer layer is a colayer, a carrier or substrate layer releasably held to said outer layer.

2. A transfer member as claimed in claim 1 wherein said gloss film comprises three layers being said inner layer, an intermediate layer and said outer layer.

3. A transfer member as claimed in claim I wherein the inner layer comprises isotactic polypropylene alone or in combination with random ethylene propylene co-polymer present in the amount of 0 to 40% by weight, and optionally additives being antistatic and slip agents present in an amount of 0 to 5% by wt., and optionally a further additive being an anti block agent present in an amount 500-4000 ppm 'by weight of isotactic polypropylene.

4. A transfer member as claimed in claim 2 wherein the intermediate layer comprises isotactic polypropylene and said additives present in the amount of 500-10000 PPM by wt. of isotactic polypropylene.

5. A transfer member as claimed in claim 1 wherein the outer layer comprises isotactic polypropylene alone or in combination with random ethylene propylene copolymer.

6. A transfer member as claimed in claims 1 to 5 wherein said antistatic and slip agents are selected from erucamide stearamide, silicon oil, stearic acid and stearates used alone or in any combination thereof, said antiblock agents selected from silica, silicate clay, talc and quartz alone or in any combination thereof.

7. A transfer member as claimed in claim I wherein the thickness each of said inner and outer layer is 2-8 x 10⁻⁶ m (2 to 8 microns).

8. A transfer member as claimed in claim 1 wherein the thickness of said member is 8-45 x 10⁻⁶ m (8 to 45 microns).

9. A transfer member as claimed in claim 1 comprising a foil provided on said film, said foil selected from a print, colour or metallized foil.

10. A transfer member as claimed in claim 9 wherein each of said foils comprise a plurality of layers with at least an outermost layer being an adhesive layer adapted to contact the leather surface and inner most layer being a release layer in contact with the film and an active layer provided therebetween, and wherein the active layer is either a print, colour or metallized layer.

11. A transfer member as claimed in claim 10 wherein the print and colour foil has each a feel modifier layer comprising a plurality of layers and wherein one of the layers is a feel modifier layer and the other layer is a top coat layer or a cover coat layer.

12. A transfer member as claimed in claim 10 wherein the print and colour foil has each a feel modifier layer comprising a plurality of layers and wherein one of the layers is a feel modifier layer adjacent to the release coat, a top coat layer adjacent to the feel modifier layer, and a cover layer adjacent to the top coat layer.

13. A transfer member as claimed in claim 10 wherein the metallized foil includes a top coat layer on said release coat layer.

14. A transfer member as claimed in claims 11 and 12 wherein the feel modifier comprises a combination of or only a single wax such as microcrystalline wax, paraffin, natural or synthetic waxes in solution or emulsion form.

15. A transfer member as claimed in claims 11 and 12 wherein the feel modifier layer also comprises oils used singularly or in combination with polydialkyl siloxane, olein modified siloxanes, diethylene modified silicon oils, epoxy modified silicon oils alcohol modified silicon oils.

16. A transfer member as claimed in claims 11 and 12 wherein the feel modifier layer comprises combination of waxes and lubricants of separate layers of waxes and lubricants.

17. A transfer member as claimed in claim 11 to 13 wherein the top coat layer comprises lacquer and lacquer emulsions of various resins, such as nitrocellulose copolymer of vinyl chloride and vinyl acetate, polyurethane and polyamides with or without cross linking agents with or without fillers, such as silica.

18. A transfer member as claimed in claims 11 and 12 wherein the cover coat layer comprises essentially of natural resins such as shellac, caesin, albumin and gelatine or plasticizers.

19. A transfer member as claimed in claims 11 and 12 wherein the cover coat layer comprises synthetic resins such as acrylic, methacrylic, synthetic rubber, vinyl resin, nitrocellulose resins or polyurethane or a combination of said natural and synthetic resins.

20. A transfer member as claimed in claims 11 and 12 wherein the cover coat layer may also include colourants with or without dispersing agents, with or without cross linking or curing agents.

21. A transfer member as claimed in claim 13 wherein a print coat layer is between said metallized layer and top coat layer.

## Patentansprüche

1. Ein Transferelement, um Leder Glanzeigenschaften zu verleihen, mit einem Glanzfilm aus wenigstens zwei koextrudierten Schichten, wobei die innere Schicht die aktive oder Glanzschicht ist und die äußere Schicht eine Zusatzschicht, einer Träger- oder Substratschicht, die lösbar an der genannten äußeren Schicht gehalten ist.

2. Ein Transferelement gemäß Anspruch 1,
wobei der genannte Glanzfilm drei Schichten umfasst, die die genannte innere Schicht, eine Zwischenschicht und die genannte äußere Schicht sind.

3. Ein Transferelement gemäß Anspruch 1,
wobei die innere Schicht isotaktisches Polypropylen allein oder in Kombination mit einem beliebigen Ethylenpropylen-Copolymer enthält, das in der Menge von 0 bis 40 Gewichts-% vorliegt, und optional Additiven die Antistatik- und Gleitmittel sind, die in einer Menge von 0 bis 5 Gewichts-% vorliegen, und optional einem weiteren Additiv, das ein Antiblockmittel ist, das in einer Menge von 500 - 4000 ppm nach Gewicht von isotaktischem Polypropylen vorliegt.

4. Ein Transferelement gemäß Anspruch 2,
wobei die Zwischenschicht isotaktisches Polypropylen enthält und die genannten Additive, die in der Menge von 500 - 10000 ppm nach Gewicht von isotaktischem Polypropylen vorliegen.

5. Ein Transferelement gemäß Anspruch 1,
wobei die äußere Schicht isotaktisches Polypropylen allein oder in Kombination mit einem beliebigen Ethylenpropylen-Copolymer enthält.

6. Ein Transferelement gemäß den Ansprüchen 1 bis 5,
wobei die genannten antistatischen und Gleitmittel gewählt werden von Erucamidsteramid, Siliconöl, Stearinsäure und Stearaten, die allein benutzt werden oder in jeglicher Kombination, wobei das genannte Antiblockmittel gewählt wird aus Silika, Silikalehm, Talk und Quarz alleine oder in jeglicher Kombination davon.

7. Ein Transferelement gemäß Anspruch 1,
wobei die Dicke von jeder der genannten inneren und äußeren Schichten 2 - 8 x 10⁻⁶ m (2 bis 8 Micron) ist.

8. Ein Transferelement gemäß Anspruch 1,
wobei die Dicke des Elementes 8 - 45 x 10⁻⁶ m (8 bis 45 Micron) ist.

9. Ein Transferelement gemäß Anspruch 1,
das eine Folie enthält, die auf dem genannten Film vorgesehen ist,
wobei die Folie gewählt wird aus einer Druck-, Farb- oder metallisierten Folie.

10. Ein Transferelement gemäß Anspruch 9,
wobei jede der genannten Folien eine Vielzahl von Schichten enthält, mit wenigstens einer äußersten Schicht, die eine Haftschicht ist, die angepasst ist, um die Lederschicht zu kontaktieren, und einer innersten Schicht, die eine Löseschicht in Kontakt mit dem Film ist, und einer aktiven Schicht, die dazwischen vorgesehen ist, und wobei die aktive Schicht entweder eine Druck-, Farb- oder metallisierte Schicht ist.

11. Ein Transferelement gemäß Anspruch 10,
wobei die Druck- und Farbfolie jeweils eine Gefühlveränderungsschicht haben, die eine Vielzahl von Schichten enthalten, und wobei eine der Schichten eine Gefühlveränderungsschicht ist und die andere Schicht ist eine oberste Mantelschicht oder eine Abdeckmantelschicht.

12. Ein Transferlement gemäß Anspruch 10,
wobei die Druck- und Farbfolie jeweils eine Gefühlveränderungsschicht hat, die eine Vielzahl von Schichten enthält und wobei eine dieser Schichten eine Gefühlveränderungsschicht ist, benachbart zu der Lösebeschichtung, eine oberste Mantelschicht benachbart zu der Gefühlveränderungsschicht und eine Abdeckschicht benachbart zu der obersten Mantelschicht.

13. Ein Transferelement gemäß Anspruch 10,
wobei die metallisierte Folie eine oberste Mantelschicht auf der genannten Lösemantelschicht enthält.

14. Ein Transferelement gemäß Anspruch 11 und 12,
wobei der Gefühlveränderer eine Kombination von Wachsen oder nur ein einzelnes Wachs enthält wie mikrokristallines Wachs, Paraffin, natürliche oder synthetische Wachse in Lösung oder Emulsionform.

15. Ein Transferelement gemäß Anspruch 11 und 12,
wobei die Gefühlveränderungsschicht ebenfalls Öle enthält, die einzeln oder in Kombination benutzt werden mit Polydiaekylsyloan, Olein modifizierte Syloane, Dyethylen modifizierte Siliconöle, Epoxymodifizierte Siliconöle, Alkohol-modifizierte Siliconöle.

16. Ein Transferelement gemäß Anspruch 11 und 12,
wobei die Gefühlveränderungsschicht Kombinationen enthält von Wachsen und Schmiermitteln von unterschiedlichen Schichten von Wachsen und Schmiermitteln.

17. Ein Transferelement gemäß Anspruch 11 bis 13,
wobei die oberste Mantelschicht Lack enthält und Lackemulsionen verschiedener Harze, wie Nitrozellulosecopolymer von Vinylchlorid und Vinylacetat, Polyurethan und Polyamiden mit oder ohne Vernetzungsmittel, mit oder ohne Füller wie Silicon.

18. Ein Transferelement gemäß Anspruch 11 und 12,
wobei die Abdeckmantelschicht im Wesentlichen besteht aus natürlichen Harzen wie Schellack, Kasein, Albumin und Gelatine oder Weichmachern.

19. Ein Transferelement gemäß Anspruch 11 und 12,
wobei die Abdeckmantelschicht synthetisches Harz enthält wir Acryl-, Methacryl-, synthetisches Gummi, Vinylharz, Nitrocelluloseharze oder Polyurethane oder eine Kombination der genannten natürlichen und synthetischen Harze.

20. Ein Transferelement gemäß Anspruch 11 und 12,
wobei die Abdeckmantelschicht ebenfalls Farbmittel enthalten kann mit oder ohne Dispergiermittel, mit oder ohne Vernetzungs- oder Aushärtmittel.

21. Ein Transferelement gemäß Anspruch 13,
wobei eine Druckmantelschicht zwischen der genannten metallisierten Schicht und der obersten Mantelschicht ist.

## Revendications

1. Élément de transfert destiné à donner des propriétés de brillance au cuir, comprenant un film brillant d'au moins deux couches co-extrudées et dans lequel la couche interne est la couche active ou brillante et la couche externe est une couche associée, une couche porteuse ou une couche support maintenue de façon amovible sur ladite couche externe.

2. Élément de transfert selon la revendication 1 dans lequel ledit film brillant comprend trois couches qui sont la couche interne, une couche intermédiaire et ladite couche externe.

3. Élément de transfert selon la revendication 1 dans lequel la couche interne comprend du polypropylène isotactique seul ou combiné à un copolymère aléatoire éthylène propylène présent dans une proportion comprise entre 0 et 40 % en poids, et en option des additifs qui sont des agents antistatiques et de glissance présents dans une proportion comprise entre 0 et 5 % en poids, et en option un autre additif qui est un agent antiadhérent présent dans une quantité comprise entre 500 et 4000 ppm en poids de polypropylène isotactique.

4. Élément de transfert selon la revendication 2 dans lequel la couche intermédiaire comprend du polypropylène isotactique et lesdits additifs présents dans une quantité comprise entre 500 et 10 000 ppm en poids de polypropylène isotactique.

5. Élément de transfert selon la revendication 1 dans lequel la couche externe comprend du polypropylène isotactique seul ou combiné à un copolymère aléatoire éthylène propylène.

6. Élément de transfert selon les revendications 1 à 5 dans lequel lesdits agents antistatiques et de glissance sont sélectionnés parmi les éléments suivants : érucamide, stéaramide, huile siliconée, acide stéarique et stéarates utilisés seuls ou en combinaison entre eux, lesdits agents antiadhérents étant sélectionnés parmi les éléments suivants : silice, argile de silicate, talc et quartz utilisés seuls ou en combinaison entre eux.

7. Élément de transfert selon la revendication 1 dans lequel l'épaisseur de chacune des dites couches interne et externe est comprise entre 2 et 8 x 10⁻⁶ m (2 à 8 microns).

8. Élément de transfert selon la revendication 1 dans lequel l'épaisseur dudit élément est comprise entre 8 et 45 x 10⁻⁶ m (8 à 45 microns).

9. Élément de transfert selon la revendication 1 comprenant une feuille sur ledit film, ladite feuille étant une feuille imprimée, une feuille de couleur ou une feuille métallisée.

10. Élément de transfert selon la revendication 9 dans lequel chacune des dites feuilles comprend une pluralité de couches, avec au moins une couche adhésive occupant la position externe extrême adaptée à un contact avec la surface du cuir et une couche anti-adhésive occupant la position interne extrême en contact avec le film, et une couche active entre les deux, et dans lequel la couche active est une couche imprimée, une couche colorée ou une couche métallisée.

11. Élément de transfert selon la revendication 10 dans lequel la feuille imprimée et la feuille colorée ont chacune une couche de modification de toucher comprenant une pluralité de couches et dans lequel l'une des couches est une couche de modification de toucher et l'autre couche est une couche de finition ou une couche de couverture.

12. Élément de transfert selon la revendication 10 dans lequel la feuille imprimée et la feuille colorée ont chacune une couche de modification de toucher comprenant une pluralité de couches et dans lequel l'une des couches est une couche de modification de toucher adjacente à la couche anti-adhésive, une couche de finition adjacente à la couche de modification de toucher et une couche de couverture adjacente à la couche de finition.

13. Élément de transfert selon la revendication 10 dans lequel la feuille métallisée est une couche de finition sur ladite couche anti-adhésive.

14. Élément de transfert selon les revendications 11 et 12 dans lequel le modificateur de toucher comprend une seule cire, ou une combinaison de cires, telle(s) que la cire microcristalline, la paraffine, des cires naturelles ou synthétiques sous forme de solution ou d'émulsion.

15. Élément de transfert selon les revendications 11 et 12 dans lequel la couche de modification de toucher comprend également des huiles utilisées seules ou en combinaison avec du siloxane polydialkyle, des siloxanes modifiés par l'oléine, des huiles siliconées modifiées par le diéthylène, des huiles siliconées modifiées par l'époxy, des huiles siliconées modifiées par l'alcool.

16. Élément de transfert selon les revendications 11 et 12 dans lequel la couche de modification de toucher comprend une combinaison de cires et de lubrifiants issus de couches séparées de cires et de lubrifiants.

17. Élément de transfert selon les revendications 11 à 13 dans lequel la couche de finition comprend une laque et des émulsions de laque de diverses résines, telles qu'un copolymère de nitrocellulose de chlorure de vinyle et d'acétate de vinyle, du polyuréthane et des polyamides avec ou sans agents de réticulation avec ou sans charges, telles que la silice.

18. Élément de transfert selon les revendications 11 et 12 dans lequel la couche de couverture se compose essentiellement de résines naturelles telles que la gomme laque, la caséine, l'albumine et la gélatine ou des plastifiants.

19. Élément de transfert selon les revendications 11 et 12 dans lequel la couche de couverture se compose de résines synthétiques telles que résine acrylique, résine méthacrylique, caoutchouc synthétique, résine vinylique, résines nitrocellulose ou polyuréthane ou une combinaison des dites résines naturelles et synthétiques.

20. Élément de transfert selon les revendications 11 et 12 dans lequel la couche de couverture peut également inclure des colorants avec ou sans agents dispersants, avec ou sans agents de réticulation ou de polymérisation.

21. Élément de transfert selon la revendication 13 dans lequel une couche imprimée est disposée entre ladite couche métallisée et la couche de finition.
